

## UNITED STATES PATENT OFFICE

2,352,810

## GRAINING INK VEHICLE

Raymond A. Swain, Bellevue, Ky., assignor to Interchemical Corporation, New York, N. Y., a corporation of Ohio

No Drawing. Application May 17, 1941,  
Serial No. 393,927

3 Claims. (Cl. 260—22)

This invention relates to the art of artificial woodgraining, and it is particularly directed to new vehicles useful in the preparation of graining inks, and to graining inks containing these vehicles.

The usual method of reproducing grain patterns of fine woods on either cheap wood or metal is, first, to apply a base coat, or ground coat, to the surface to be "grained" which hides the true appearance of the surface and provides a background color for the grain design. This is printed with the grain pattern by means of a resilient roll bearing the graining ink in the desired pattern from contact with an intaglio cylinder. After the graining ink has dried, a covering of a clear varnish or resinous composition, tinted with a transparent color if desired, is applied to protect the printed graining and to provide a finish resembling genuine wood finishes. Sometimes, when applying an artificial grain to wood, the ground coat may be omitted and the graining ink applied directly to the bare wood.

Graining inks must have certain physical characteristics which distinguish them from the ordinary intaglio printing inks. In the case of wood graining inks where no ground coat is employed, the ink must not bleed or run noticeably along the fibers and pores of the wood, and yet it is desirable that the ink be completely absorbed by the wood and feather out slightly on coming in contact therewith in order to obtain a clear but pleasingly soft appearing grain. Where the graining ink is applied over a ground coat, especially in coating metal, it is essential that the ink should bond well to the ground coat, which means that the solvents in the ink should not deleteriously affect the ground coat. That is, the graining ink should not cause either embossing or shelving (i. e. separation of the various films or coats). Likewise, the ink should be capable of bonding well with the top coats of clear lacquer or resin.

This invention provides new vehicles for graining inks more nearly embodying the desired physical properties enumerated above than graining ink vehicles known in the prior art. Graining inks formulated with these vehicles will bond tightly to all of the usual ground and top coatings without shelving or embossing and they may be retouched. The invention also includes the graining inks formulated with these vehicles.

The vehicles of this invention may be broadly defined as condensation products of phthalic anhydride (or acid), glycerol, benzoic acid and drying or semi-drying oil fatty acids, containing a

plasticizer (and solvent if necessary) intimately admixed therewith.

The solvent or plasticizer preferably should have a fairly high boiling point in order that it may not evaporate from the graining ink but remain in the dried or hardened ink after it has been applied to the surface to be decorated. Generally, this requires that the plasticizer have a boiling point of at least 350° F., and where the graining ink is to be baked on the decorated surface the plasticizer should have an even higher boiling point. Some of the most suitable plasticizers are the dialkyl esters of phthalic acid, and of these dimethyl phthalate is preferred.

Since such heavy plasticizers often increase the viscosity of the graining ink or paste undesirably, it is often preferable to dilute the plasticizer with a lower boiling solvent which will evaporate to a large extent on application of the graining ink to decorated surfaces. Very volatile solvents are to be avoided as they will evaporate from the ink during exposure on the intaglio printing rolls with the result that the ink becomes nonuniform in composition. Solvents which are generally quite satisfactory are those whose boiling points are above that of water, but not greatly beyond, and it has been found that methyl ether of ethylene glycol (methyl cellosolve) is particularly suitable as a solvent in connection with dimethyl phthalate as a plasticizer.

Although any of the commercially available drying and/or semi-drying oil fatty acids may be used in preparing these vehicles, soya bean, tung and perilla fatty acids give products having the desired physical properties to a greater degree than do the products of other drying oil acids. It is obvious, of course, that the drying oils themselves may be substituted in part for the equivalent amounts of glycerin and drying oil fatty acids, and such choice is within the discretion of those skilled in the art.

The preparation of a typical graining ink vehicle according to this invention is described in the following example, in which the materials are given in parts by weight.

## Example 1

|                       | Parts by weight |
|-----------------------|-----------------|
| Phthalic anhydride    | 351             |
| Glycerol              | 236             |
| Benzoic acid          | 134             |
| Soya bean fatty acids | 269             |
| Dimethyl phthalate    | 606             |

The phthalic anhydride, glycerol, benzoic acid and soya bean fatty acids were heated together in

a kettle to 450° F. and maintained at that temperature for two and one half hours in an atmosphere of carbon dioxide. After the acid number of the mixture had dropped to 14 the batch was cooled down and the dimethyl phthalate slowly added with constant mixing.

This vehicle showed compatibility with nitrocellulose, alkyd resins, maleic gums and the like. Generally, graining inks made with this vehicle are more suitable for use over the baked type of ground coats because the dimethyl phthalate may have a deleterious effect on the air dried type, due to penetration into the ground coat.

Typical graining inks employing the vehicle described in Example 1 are as follows, in which the materials are given in parts by weight:

*Example 2—Transparent graining ink*

|                      | Parts by weight |
|----------------------|-----------------|
| Blanc fixe           | 30.00           |
| Vehicle of Example 1 | 22.50           |
| Dimethyl phthalate   | 7.50            |

The above materials were mixed and ground on a roll mill to a uniform paste. Then an additional 30.00 parts of the vehicle and 10.00 parts of dimethyl phthalate were added and the mixture ground until a completely uniform and smooth paste or graining ink was obtained.

*Example 3—White graining ink*

|                      | Parts by weight |
|----------------------|-----------------|
| Titanium dioxide     | 56.10           |
| Vehicle of Example 1 | 32.90           |
| Dimethyl phthalate   | 11.00           |

The materials were ground on a roll mill until a uniform paste was obtained.

*Example 4—Mahogany graining ink*

|                      | Parts by weight |
|----------------------|-----------------|
| Madder lake          | 9.10            |
| Carbon black         | 5.50            |
| Bone black           | 8.80            |
| Burnt sienna         | 3.60            |
| Vehicle of Example 1 | 54.75           |
| Dimethyl phthalate   | 18.25           |

The materials were ground together on a roll mill until the resulting paste was of uniform consistency.

*Example 5—Walnut graining ink*

|                        | Parts by weight |
|------------------------|-----------------|
| Burnt umber            | 19.75           |
| Raw sienna             | 18.20           |
| Carbon black           | 0.70            |
| Vehicle from Example 1 | 46.00           |
| Dimethyl phthalate     | 15.35           |

The materials were ground on a roll mill as described in Example 4.

All of these graining inks will air dry, usually

in a couple of hours, but they may be dried in a relatively few minutes by baking at temperatures up to about 300° F., the only limitation being the sensitivity of the contained pigments to discoloration by heat.

Although these graining inks may be applied to wood directly, it is generally desirable to apply a ground coat first. The ground coat may be any of the compositions usually employed for this purpose and which are hardened by baking, such as alkyd and urea resins, and ground coats containing an alkyd resin binder are especially suitable.

Similarly, any of the standard top coating compositions may be applied over the graining ink, and the clear nitrocellulose lacquers or clear finishes made from maleic gums, urea resins and the like, are suitable.

It is understood that wherever phthalic anhydride is referred to in the specification and claims its obvious equivalent, phthalic acid, may be substituted, and it is included within the scope of the claims. Likewise, mixtures of fatty acids or drying and semi-drying oils may be used in place of the fatty acids derived from a single drying oil.

I claim:

1. A graining ink having correct body for intaglio offset application, comprising coloring matter dispersed in a vehicle consisting essentially of an alkyd resin and a solvent therefor having a boiling point above that of water, and a substantial portion thereof being a plasticizer for the resin boiling above 350° F., whereby substantial change of ink body during application is avoided, in such quantity that correct body is attained, the resin being a reaction product of phthalic anhydride and glycerol modified with both benzoic acid, and fatty acids derived from oils selected from the group consisting of drying and semi-drying oils.

2. A graining ink having a body designed for intaglio offset application, comprising coloring matter dispersed in a vehicle consisting essentially of the reaction product of glycerol, phthalic anhydride, benzoic acid and soya oil fatty acids, reduced to graining ink consistency with dimethyl phthalate.

3. A graining ink having a body designed for intaglio offset application, comprising coloring matter dispersed in a vehicle consisting essentially of the reaction product of approximately 24 parts by weight of glycerol, approximately 35 parts by weight of phthalic anhydride, approximately 13 parts by weight of benzoic acid, and approximately 27 parts by weight of soya oil fatty acids, reduced to graining ink consistency with dimethyl phthalate.

RAYMOND A. SWAIN.